

# UNITED STATES PATENT OFFICE.

JEAN ROSEN, OF PARIS, FRANCE, ASSIGNOR TO SOCIÉTÉ ANONYME DES COMBUSTIBLES INDUSTRIELS, OF PARIS, FRANCE.

## PROCESS OF MANUFACTURE OF IMPREGNATED MATERIAL.

1,155,443.

Specification of Letters Patent.

Patented Oct. 5, 1915.

No Drawing.

Application filed July 22, 1914. Serial No. 852,516.

*To all whom it may concern:*  
Be it known that I, JEAN ROSEN, a citizen of France, residing at 25 Rue Pigalle, Paris, France, have invented certain new and useful Improvements in Processes of Manufacture of Impregnated Material, of which the following is a specification.

This invention relates to a process of manufacture of an unalterable and insulating impregnating material and application of same.

The present process may involve the use of the process of my pending application Serial Number 783,814, or important steps thereof.

The process of this invention consists in the manufacture of a perfectly impermeable material that is both insulating and unalterable, and comprises the application of this material on all kinds of rigid or flexible supports to be used as water-tight or nonconducting supports or for electric insulation and the like.

The raw material consists of coal tar and its various neutral liquid and heavy constituents that by distillation or partial oxidation under suitable conditions are made to undergo a physico-chemical transformation so as to obtain an elastic impermeable, perfectly insulating material that resists for an almost indefinite length of time to the natural causes of alteration and becomes soft only at a comparatively high temperature.

The tar is first heated so as to remove by known methods the caustic substances and a part of the crystallizable easily volatilized products that it normally contains (phenols, naphthalene, etc.). The liquid and heavy products for instance, water, naphthalene, naphthalene oils, creosote and creosote oils, carried over during this elimination are separated by known means (such as by one or more of the steps of sublimation, crystallization, and treatment with chemical reagents,) from the light and caustic products and the crystalline substances mixed therewith. The liquid, heavy and non-caustic or neutral constituents separated in this manner are then partly mixed with the residuary exhausted tar and the whole is then submitted to an oxidizing current of air, that is used in a moderate proportion and at such a temperature that the transformation by oxidation is obtained almost quantitatively. The treatment by oxidation must be kept up

until the product obtained has the consistency and properties required: *i. e.*, until it has acquired a high degree of resiliency and a high softening point and has been rendered unalterable by chemical reagents or the action of the atmosphere. The insulating and plastic material obtained in this manner and melted at a high temperature can then be used for impregnating by steeping or coating any permeable substratum such as paper, card board, felt, tissue of any kind, porous terracotta, etc., that is thoroughly penetrated by the insulating material. The support chosen which may be rigid or flexible but must be permeable, is impregnated according to its nature and that of the tar treated, with the liquid, neutral and heavy constituents that were separated off during the first treatment above referred to, part of these constituents having been put aside for this purpose. The excess of these substances is carefully eliminated by compression and wiping off and the supports prepared in this manner are submitted to the action of the impregnating substance, that has been oxidized in the manner referred to and brought to a high temperature. After impregnating, the support is cooled and further oxidized preferably by means of currents or jets of air.

The process of manufacture and application of the same offers the following advantages over the old methods:—the perfect penetration of the insulating substance into the porous material used as a support; the great elasticity of the product so that without breaking it can undergo the most abrupt deformations to which the non rigid supports may be subjected; the unalterable nature of the coating for an almost indefinite length of time; the resistance to atmospheric action and chemical reagents without any marked tendency to become brittle when cold or sticky when hot; the possibility of impregnating the paper, felt, tissue of any kind, etc., on both sides without subsequently causing the surfaces rolled up or brought in contact with one another to stick even under high pressure and in the absence of an accessory absorbent such as talc, sand, canvas with large meshes and the like.

What I claim is:

1. A process for the manufacture of an unalterable elastic and insulating impreg-

nating product and impregnating supporting material consisting in treating coal tar by heating to remove its caustic and easily volatilizable crystalline substances, adding neutral oil to the tar, oxidizing the mixture by air, coating the support material with the product, and subsequently cooling the final product with air.

2. A process for the manufacture of an unalterable elastic and insulating impregnating product and impregnating supporting material consisting in treating coal tar by heating to remove its caustic and easily volatilizable crystalline substances, by heating and adding to the residue heavy neutral oil, thereupon submitting the mixture of tar

residue and oil obtained to the oxidizing action of air, impregnating the supporting material by steeping said material in the oxidized insulating and plastic product obtained while heating the latter, and subsequently cooling the product by a current of air so as to cause the impregnating product to oxidize and solidify owing to the comparatively high temperature of solidification of this impregnating product.

In testimony whereof I affix my signature in presence of two witnesses.

JEAN ROSEN.

Witnesses:

CHAS. P. PRENBY,  
FELIX MOULISON.

Copies of this patent may be obtained for five cents each, by addressing the "Commissioner of Patents, Washington, D. C."